

# UNITED STATES PATENT OFFICE.

ARRIGO TEDESCO, OF TURIN, ITALY, ASSIGNOR TO SOCIETA ANONIMA STABILIMENTI BIAK, OF TURIN, ITALY, A COMPANY OF ITALY.

## ALLOYS HAVING HIGH MECHANICAL, CHEMICAL, AND ELECTRICAL RESISTANCE.

1,351,811.

Specification of Letters Patent.

Patented Sept. 7, 1920.

No Drawing.

Application filed March 6, 1919. Serial No. 281,084.

To all whom it may concern:

Be it known that I, ARRIGO TEDESCO, subject of the King of Italy, and resident of Turin, Italy, have invented certain new and useful Improvements in Alloys Having High Mechanical, Chemical, and Electrical Resistance, of which the following is a specification.

This invention has for its object the production of a copper-nickel alloy having certain marked characteristics, and particularly good technological characteristics, associated with a high resistance to the chemical action of a number of acids.

The alloy according to the invention is a nickel-copper alloy and consists of nickel in proportion amounting to nearly one half of the final alloy, a portion of the copper being exchanged for iron and a portion for a rare metal such as tungsten or titanium.

The percentage of the metals forming the alloy may vary within the limits set forth below, according to the particular use for which the alloy is intended:

Copper, from 35 to 44 per cent.  
Iron, from 1.5 to 4.75 "  
Tungsten, from 3 to 6 "  
Nickel, the rest.

By way of example the following composition may be given as constituting an alloy in accordance with the invention:

|          |              |
|----------|--------------|
| Copper   | 40 per cent. |
| Iron     | 3 "          |
| Tungsten | 3 "          |
| Nickel   | 54 "         |

Alloys of such composition, in cast condition, have a tensile strength of about 55 kilos per sq. mm. and an elongation of about 20 per cent.; they may be forged and rolled both cold and hot. After drawing in some cases the tensile strength exceeds 100 kilos per sq. mm.

An alloy of the type described shows a resistance to the flow of electric current of

about 0.600—10<sup>4</sup> and has a very strong resistance to the corrosive action of a number of acids.

In fact, a plate made with an alloy according to this invention, exposed for 12 hours to the action of sulfuric acid of 15° Bé. at a temperature of 50° C. has not been corroded; this plate treated for the same time with sulfuric acid of 50° Bé. at a temperature of 50° C. has shown a weight reduction of about 0.90 milligram per sq. cm. Generally speaking, this alloy is satisfactorily resistant to sulfuric acid of any strength and, at temperatures under 100° without being materially corroded.

The resistance of the alloy to a number of other acids is hereinafter mentioned:

Hydrochloric acid: The alloy resists this acid in any strength and at any temperature;

Acetic acid: As above;

Citric acid: As above;

Tannic acid: As above;

Nitric acid: The alloy resists satisfactorily the action of cold nitric acid up to a concentration of 1.49 Bé.

The alloy also has a satisfactory resistance to nitro-sulfuric acid.

Therefore these alloys are particularly adapted for cases in which is required a high resistance to chemical action as well as either a high resistance to mechanical stresses or a high electrical resistance or both.

What I claim and desire to secure by United States Letters Patent is:

An alloy having high mechanical, chemical and electrical resistance, comprising nickel in proportion of about one half of the final alloy, copper in proportion between 35 and 44 per cent. iron in proportion between 1.5 and 4.75 per cent. and tungsten in proportion between 3 and 6 per cent.

Signed at Turin, Italy, this 11th day of February A. D. 1919.

ARRIGO TEDESCO.